

## UNITED STATES PATENT OFFICE

ROBERT JAY SHOEMAKER, OF CHICAGO, ILLINOIS, ASSIGNOR TO S. & T. METAL COMPANY, OF CHICAGO, ILLINOIS, A CORPORATION OF ILLINOIS

## BEARING METAL

No Drawing. Application filed September 16, 1927, Serial No. 220,062. Renewed November 8, 1929.

This invention relates to the production of lead base alloys, and its object is to produce a lead alloy of such character that it may be used for bearings, bushings or other like elements where anti-friction surfaces are required or for other purposes where a hardened lead is desirable. The invention has particularly in view the production of an anti-friction metal which will be tough and relatively hard so as to be capable of supporting heavy loads, and which at the same time possesses lubricating properties.

A further object of the invention is to provide an alloy of this character, the alloying metals of which will not drop or burn out, at least to any undesirable extent, either when the ingredient metals are melted together in compounding the alloy, or when the alloy is melted in casting operations.

20 A further object is to provide an alloy of this character, which because of the character of its ingredients and its method of manufacture can be economically produced.

The invention consists essentially in the use of a very small quantity of lithium as a hardening agent, sometimes in combination with a larger quantity of sodium, and the use with these materials of small quantities of calcium and aluminum to facilitate the combination and to prevent drossing. Although lithium is a comparatively expensive metal, it has been discovered that the use of this metal in extremely small quantities (as little as .01 to .05%) will greatly increase the hardness of the alloy and in such small quantities

this metal may be economically used. It is also effective in combination with sodium which is much cheaper and may be used in comparatively larger quantities. The lead alloy into which these metals have been introduced will be extremely unstable and the rare elements will burn or boil out, unless calcium and aluminum are used as anti-drossing agents, the use of both of these metals being practically necessary for reasons set forth hereinafter.

The following example will serve to illustrate the principles governing the compounding of this alloy. Modifications will be suggested and these modifications and all em-

bodiments of the invention within the scope of the appended claims are intended to be covered by the patent.

The alloy may be composed of the following metals in substantially the proportions which follow:

|          |                 |
|----------|-----------------|
| Lithium  | .01% to .05%    |
| Sodium   | .2% to .8%      |
| Calcium  | .1% to .7%      |
| Aluminum | .02% to .1% 60  |
| Tin      | 1% to 2%        |
| Lead     | to make up 100% |

The base metal is first produced by heating lead in a crucible to about 1600° Fahrenheit, 65 the lead bath then being covered with calcium chloride or other suitable substance which will fuse and float on the molten metal without burning at the temperature specified. Metallic calcium is then stirred into the melt 70 while covered with a supernatant covering of calcium chloride, which prevents the calcium from burning by exclusion of oxygen. The tin and aluminum are introduced in the same manner, the molten alloy thoroughly 75 mixed, and then cast into ingots.

The ingots are then remelted to 650° to 700° Fahrenheit and the bath covered with rosin or other neutral flux. The metallic sodium is then stirred in. The lithium is introduced as a lithium lead alloy, or in the form of metallic lithium. The lithium may also be introduced by electrolyzing a lithium-halogen salt using molten lead as one electrode.

85 The lithium is the primary hardening agent, and .05% or less of lithium will serve to increase the hardness of the alloy to from 23 to 30° Brinnell. The sodium is also a hardening agent, and since it is much cheaper than lithium it may be used in larger quantities, and it has been found that the lithium and sodium combination above set forth is more effective as a hardening agent in proportion to the quantity used than either 90 of the elements used alone.

The lithium and sodium form very unstable combinations and will burn or boil out unless anti-drossing agents are used, and this is the primary function of the calcium and alumi- 100

num. A film of calcium hydroxide is formed on the molten alloy which serves to protect the rarer metals and hold them in the combination. The aluminum coacts with the calcium to keep down the amount of calcium which separates out and to minimize the drossing loss of the other materials, particularly when the alloy is remelted.

It seems that neither the calcium nor 10 aluminum alone are sufficient to adequately prevent the loss of the lithium, but that the two must be used together as specified, unless exceptional care is taken in preparing small quantities of the alloy at a time. The 15 use of tin is optional but preferable, and its use serves as an easy way to introduce the aluminum in the form of an aluminum-tin alloy.

It has been found that alloys compounded 20 substantially as hereinabove set forth are strong, tough and of adequate hardness, while still possessing all of the lubricating qualities of a good bearing metal. Since the lithium is used only very small quantities, the expense 25 of the materials is not unduly increased, and the combined use of calcium and aluminum as anti-drossing agents makes the alloy easy to compound and remelt without serious loss of the essential constituents.

30 I claim:

1. A lead base alloy containing the following metals in approximately the proportions, by weight, as follows: lithium .01 to .05%, sodium .2 to .8%, calcium .1 to .7%, tin 1 to 35 2%, aluminium .02 to .1% and lead to make up 100%.

2. A lead alloy containing the following metals in approximately the proportions by weight as follows: lithium .01% to .05%, sodium .2% to .8%, calcium .1% to .7%, aluminium .02% to .1%, and lead to make up 100%.

40 ROBERT JAY SHOEMAKER.

45

50

55

60